

May 18, 1943

A. JENKNER

2,319,326

PROCESS OF PRODUCING BITUMEN-LIKE MATERIALS FROM COAL

Filed Oct. 15, 1940

2 Sheets-Sheet 1



Inventor:  
ADOLF JENKNER  
by his attorneys  
Howson and Howson

May 18, 1943

A. JENKNER

2,319,326

PROCESS OF PRODUCING BITUMEN-LIKE MATERIALS FROM COAL

Filed Oct. 15, 1940

2 Sheets-Sheet 2



Inventor:  
ADOLF JENKNER  
by his attorneys  
Hawson and Hawson

## UNITED STATES PATENT OFFICE

2,319,326

## PROCESS OF PRODUCING BITUMENLIKE MATERIALS FROM COAL

Adolf Jenkner, Wanne-Eickel, Germany; vested in the Alien Property Custodian

Application October 15, 1940, Serial No. 361,317  
In Germany October 6, 1939

12 Claims. (Cl. 196—14)

The invention relates to the production from coal of bitumen-like materials, i. e., substances of a colloidal character similar to that of the mineral oil bitumen.

According to the invention the coal in pulverulent condition is heat-treated with solvents—namely, hydrocarbon oils having a high boiling point; then part of the solvent is distilled without separation of the undissolved proportions.

The result is a bitumen-like residue which may be used for varying purposes, particularly as a substitute for bitumen used heretofore for the insulation of pipes.

It is known to extract coal with hydrocarbon oils having a high boiling point, to separate the undissolved matter after the extraction and to distill solvents, if necessary. In this manner it was possible to produce pitch-like materials which, however, differ materially from the product made in accordance with the invention.

It was also known to heat coal with tar to comparatively high temperatures, namely to such temperatures where a decomposition of the coal occurs, and then to use the obtained product without separating the solid substances. Also this known process results in products which differ from those made in accordance with the invention, in the same manner as the processes for making fluent coal where coal with oils is worked into a stable suspension.

With all of these known processes, the production of bitumen-like substances was neither intended nor achieved.

In solving this problem, a number of process conditions must be observed to obtain the result desired.

Thus it has been found that a bitumen-like product cannot be made from every mineral coal, but that it is necessary to use glance coal otherwise known as anthracite or a coal consisting for the greater part of glance coal, using preferably coal possessing baking properties.

It has also been found that the result desired can only be obtained if the initial coal is subjected to the treatment with the solvent in a very pulverulent shape or if the conversion into this pulverulent shape takes place before the completion of the heat treatment in the presence of the hydrocarbon oils.

The size of particles must be less than 0.5 mm. As treating agents according to the invention, hydrocarbon oils may be used, chiefly coal tar oils, such as, for instance, anthracene oil.

It is recommended to use these oils in excess,

since otherwise overheating will hardly be avoided, which would result in disturbing decompositions. Suitably a considerable surplus of liquid treating agents is used and, e. g., a ratio in weight of oil to coal of 5 to 1 is used. Part of the oil may be added in the course of the process.

If a coking glance coal having a grain size of, say, 0.1 mm. is treated with the five- to sixfold amount of anthracene oil at temperatures where a decomposition of the coal cannot take place—e. g., at temperatures of 360° C.—for about 3 or 4 hours and then about one half is distilled without being separated from the undissolved matter at ordinary pressure, a bituminous product showing surprisingly good properties will be obtained.

The effect occurring with the process of the invention may be accounted for by the supposition that the individual particles of coal swell up in the oil without undergoing decomposition.

The temperature of treatment must be chosen in such a manner as to prevent decomposition of the coal, but—on the other hand—it must not be too low, as otherwise the desired bitumen-like state which must be considered a colloidal solution of coal in the treating agent will not be obtained or will be imperfect.

The optimum temperature of treatment for each individual case can be easily ascertained by simple preliminary tests, also the time of treatment which is suitable in the individual case and this varies slightly depending on the temperature used and the initial material. The time of treatment must be chosen of such length that the final product obtained shows the desired colloidal properties. To exceed the time of treatment involves no risk, since no reversion will take place if care is taken to avoid overheating.

To remove the used surplus of solvent, it is necessary to distill this excess solvent after the heat treatment, when care must be taken again that decompositions are avoided.

The use of vacuum or other costly means of distillation is not necessary, as has been found out.

Depending on the desired application of the final product, a more or less great amount of solvent may be left in the final product. However, excessive amounts of the solvent must not be removed, as otherwise the colloidal nature and thus the favorable properties might be impaired. Those products have proved satisfactory which possess a ratio of coal to oil of, say, 1:2 or 1:3.

When using vacuum with the distillation one will succeed in removing a greater amount of

solvent without impairing the properties of the final product and without affecting the colloidal nature.

In its behavior the final product resembles the mineral oil bitumen, especially the softening point and breaking point are similar to those of the bitumen, so that the great interval between these two points may be considered as useful properties of the final product obtained by the process according to the invention.

In the same manner as bitumen, the product of the present invention shows a colloidal nature. Thereby it differs materially from pitch which is of no colloidal nature and, by the way, shows a far smaller interval between the softening and breaking points.

When using the products for the insulation of pipes, this different behavior makes itself felt to advantage.

Bitumen used for the manufacture of pipes is required, for instance, to possess a softening point of 90-100° C. according to Krämer-Sarnow and a breaking point below -5° C. according to Fraasz. At least these values will be obtained in the product of bitumen made in accordance with the invention.

The special pitches made for the purposes of insulation of pipes have never attained the cited physical values; in particular these special pitches show, after the evaporation test, a breaking point mostly materially above 0° C., which renders their use impossible, for instance, in winter time.

As an example the following test report may be quoted. (Fine coal of the Consolidation Mine 3/4 Gelsenkirchen has been used):

| Mixture                                               |         |       |
|-------------------------------------------------------|---------|-------|
| Content of ash                                        | percent | 7     |
| Volatile constituents                                 | do      | 29    |
| Baking capacity                                       |         | 200   |
| Amount of coal used                                   | grams   | 700   |
| Solvent anthracene oil according to V. f. T. quantity | grams   | 3,500 |

| Heating                                 |       |       |
|-----------------------------------------|-------|-------|
| Heating temperature                     | °C    | 22    |
| Constant temperature                    | °C    | 360   |
| Time of heating                         | hours | 1 1/2 |
| Time of heating at constant temperature | do    | 3     |

Filled amount, 1814 grams; residue of distillation, 907 grams=50%.

Properties of the same after adding a filler in the form of limestone dust:

|                                                      |               |
|------------------------------------------------------|---------------|
| Softening point according to Krämer-Sarnow           | 91° C.        |
| Softening point after evaporation                    | 95° C.        |
| Loss on evaporation                                  | 2%            |
| Breaking point according to Fraasz                   | Above -15° C. |
| Breaking point according to Fraasz after evaporation | Above -15° C. |

It has been already mentioned that the products made according to the invention are particularly adapted for the purposes of pipe insulation. If necessary, fillers may be added to them. Such materials will be used at temperatures not exceeding 180° C., since higher temperatures are likely to cause deteriorations. At these temperatures below 180° C., sometimes—especially if the products obtained in accordance with the

invention are mixed with fillers—sufficient mobility does not exist, i. e., the material has too high a viscosity, so that the necessary thickness of insulation of the pipes to be wrapped will be exceeded. Exceeding the thickness of insulation in such a manner will result in troubles, apart from the fact that unevennesses are likely to occur and useless extra consumption will be the result.

Now it has been found that the addition of coal tar, particularly high temperature tar, similar to pitch, may influence the viscosity of the bitumen-like material, even if mixed with appreciable quantities of fillers, in such a satisfactory manner that no difficulties will be encountered in the installation at temperatures of 180° C. and less, without the breaking point of the compound being reduced unduly.

With these compounds it is by no means possible to create the desired lower viscosity, say, by addition of any materials, e. g., solvents, since a product containing a high percentage of solvents shows softening points below 70°-80° C., i. e., the compound becomes so mobile that it may be used for the insulation of pipes at 180° C. and less, but it becomes useless in other respects. When proceeding in accordance with the invention, viz., when adding pitch or coal tar, the drawbacks will not be experienced. While a lowering of the breaking point cannot be avoided, the breaking points are within the range required for natural bitumens, thus the increased mobility will not be obtained at the expense of a great disadvantage.

According to the invention, pitch is added to the product of the process disclosed either before or simultaneously with or after the admixture of fillers, or the process may be carried out in such a manner that either tar or pitch is added in the course of the process for the manufacture of the bitumen-like materials; for instance, a mixture of pulverulent glance coal, coal tar oils and pitch may be subjected to the heat treatment disclosed in the principal patent or the addition may be made after the heat treatment and prior to the distillation of the surplus solvent.

In all instances, products showing improved properties will be obtained.

The amount of the admixture may vary within comparatively wide limits; in most cases an addition of pitch ranging from 10 to 20% will be sufficient to make the compound mobile enough at working temperatures of from 170° to 180° C.

The most suitable addition is hard pitch. Such hard pitch is mixed, preferably in a reduced shape, with a bitumen-like material obtained by the process disclosed; the admixture of filters may take place simultaneously with the addition of the hard pitch. Naturally, a uniform mixing should be striven for.

The curves shown in Figs. 1 and 2 of the drawings reveal the influence upon the viscosity of a pipe wrapping substance and the effect on the breaking point when adding different amounts of hard pitch. The viscosity is expressed by the adhesive quantity per square decimeter at 175° C. It will be noted that the viscosity is influenced to advantage without the breaking point being lowered unduly.

I claim:

1. Process for the production of bitumen-like materials, wherein glance coal or anthracite or coal consisting chiefly of glance coal is treated in a pulverulent form with coal tar oils, at increased temperatures ranging below the decomposition

temperatures of the coal, and excess solvent is distilled from the resulting product of said treatment without elimination of the solid constituents.

2. Bitumen-like product from a mixture of glance coal and a hydrocarbon oil of high boiling point, wherein said product in colloidal state shows a softening point of more than 90° C. and a breaking point of less than 0° C.

3. Process for the production of bitumen-like materials, wherein anthracite coal is ground to a particle size of from one to five-tenths millimeter and treated with from four to six times its weight of anthracene oil at a temperature of from 350° to 370° centigrade, the excess solvent oil being distilled off until its remainder is only two to three times the weight of initial coal in the final product.

4. Process for the production of insulation for pipes, wherein anthracite coal is ground to a particle size of from one to five-tenths millimeter, and treated with from four to six times its weight of anthracene oil at a temperature of from 350° to 370° centigrade, the excess solvent being distilled off until its remainder is only two to three times the weight of initial coal in the final product, and filler material is added, wherein 10 to 20% of hard pitch is added prior to addition of the filler material to reduce the viscosity but not to lower the breaking point.

5. Process for the production of colloidal, bitumen-like materials, wherein coal consisting chiefly of glance coal and of a grinding fineness of less than half a millimeter, is treated with coal tar oil at increased temperatures ranging below the decomposition temperatures of the coal, and excess coal tar oil is distilled from the resulting product of said treatment without elimination of the solid constituents.

6. Process for the production of colloidal bitumen-like materials, wherein glance coal is treated in pulverulent form with anthracene oil at increased temperatures ranging below the decomposition temperature of the coal, and excess anthracene oil is distilled from the resulting product of said treatment without elimination of the solid constituents.

7. Process for the production of colloidal bi-

tumen-like materials, wherein anthracite coal of a grinding fineness of half a millimeter is treated with a surplus of from four to six times by weight of coal tar oil at increased temperatures ranging below the decomposition temperature of the coal, and excess coal tar oil is distilled off from the resulting product of said treatment without elimination of the solid constituents.

10 8. Process for the production of colloidal bitumen-like materials, wherein anthracite coal of a decomposition temperature above 370° C. is treated in pulverulent form with coal tar oil at a temperature from 350° C. to 370° C. and excess coal tar oil is distilled off from the resulting product of said treatment without elimination of the solid constituents.

9. Process for the production of colloidal bitumen-like materials, wherein anthracite coal is treated in pulverulent form with a coal tar oil, at increased temperature ranging below the decomposition temperature of the coal, and excess solvent is distilled off until the solvent amounts to only two or three times the amount of initial coal in the final product.

20 10. Colloidal bitumen-like product from a mixture of undecomposed anthracite coal and a coal tar oil, having a softening point of more than 90° C. and a breaking point of less than 0° C.

30 11. Colloidal bitumen-like product from a mixture of undecomposed glance coal and anthracene oil, having a softening point of more than 90° C. and a breaking point of less than 0° C.

12. Process for the production of bitumen-like materials, wherein glance coal or anthracite coal consisting chiefly of glance coal is treated in pulverulent form with a coal tar oil, at increased temperatures ranging below the decomposition temperatures of the coal, and excess solvent is distilled from the resulting product of said treatment without elimination of the solid constituents, and filler material is added, wherein 10 to 20% of hard pitch is added prior to the addition of the filler material to reduce the viscosity but not to lower the breaking point, for the production of insulation for pipes.

ADOLF JENKNER.